

## UNITED STATES PATENT OFFICE

ROBERT JAY SHOEMAKER, OF CHICAGO, ILLINOIS, ASSIGNOR TO S. & T. METAL COMPANY, OF CHICAGO, ILLINOIS, A CORPORATION OF ILLINOIS

## BEARING METAL AND METHOD OF MAKING SAME

No Drawing.

Application filed April 29, 1927. Serial No. 187,702.

My invention relates to lead alloys and the object of the invention is to provide a hardened, toughened and stable alloy of lead suitable for bearings, bushings or other elements 5 where anti-friction properties are required or where, for other reasons, a hardened and toughened lead is required.

A further object is to provide a lead alloy which will not dross when melted.

10 A further object is to provide a lead alloy which will not corrode when subject to moist atmosphere.

15 A further object is to provide an alloy of this character which because of the character of its ingredients and its method of manufacture can be made very cheaply.

This application is a continuation in part of my copending application filed June 1, 1925, Serial No. 34,172.

20 The following will serve to illustrate the principles governing the compounding of the alloy of the present invention. Modifications will be suggested and these modifications and 25 all embodiments of the invention within the scope of the appended claims are intended to be covered by the patent.

The alloy consists of lead, sodium, calcium, aluminum, together with tin which is optional.

30 In this alloy the primary hardening agent is the sodium. If the sodium is used in amounts greater than 0.6% the hardness will increase but also the brittleness of the alloy

35 which may make it undesirable for some uses. The anti-friction qualities, however, are not impaired, but rather improved by increasing the sodium content. The main difficulty in increasing the quantity of sodium

40 used is that the alloy will have an increased tendency to dross when melted, for example in casting the bearings or other articles for which the alloy is used, and will have an increased tendency to corrode when in contact with moisture.

45 While the sodium may be used in any amount up to 1.0% the safe and practical upper limit is probably about 0.8% and with this quantity of sodium, 50 the other ingredients remaining the same as

above specified, the hardness of the alloy will be approximately 25° Brinnell.

The primary function of the calcium is to keep the sodium from drossing out, although calcium also acts to some extent as a hardener 55 for the lead. There will be a certain loss of calcium due to oxidation in melting and remelting and the amount used should depend to some extent upon this loss. As the amount of calcium used is increased, the hardness and brittleness of the alloy is increased. 60 The calcium, if used in excess, also increases viscosity when the metal is in the molten state, which necessitates a higher pouring temperature. Apparently the calcium and the lead combine and the resultant compound crystallizes out at about 700° F. This reaction between calcium and lead probably takes place even when small amounts of calcium are 65 formed, but under these circumstances the reaction is on a small scale and may be regarded as practically negligible. The calcium can be used in even smaller amounts than 0.1% but this involves a very careful handling of the metals in process. Otherwise the sodium will dross out when the alloy 70 is melted.

The aluminum, if used in larger quantities than above specified, will produce no beneficial effect and no effect at all except that as it 80 will not go into solution in quantities above 0.1% its presence in excess of that amount tends to make the metal viscous.

The tin ingredient, which is optional, may 85 be increased very considerably, for example up to 5% or possibly 10%, but tin is also a hardener, in the compound specified, so that as the tin content is increased the resultant alloy becomes increasingly hard and increasingly brittle. The preferred limits of the tin are from 1.0% to 5.0%. A compound with the ingredients, except tin, in the proportions as above stated but with the tin 90 forming 5% of the compound, will have a hardness of approximately 23° Brinnell.

The tin may be used in amounts less than 1%, the alloy being in such case a trifle softer, or this ingredient may be omitted entirely. 100

As an example, the ingredients may be in the following proportions:

Sodium, preferably 0.7% or less but not in excess of \_\_\_\_ 1.0 %  
5 Calcium \_\_\_\_\_ 0.1 % to 0.25%  
Aluminum \_\_\_\_\_ 0.02% to 0.1 %  
Lead to make up 100%

By using a low sodium content as suggested 10 above, 0.7% or lower, with the other ingredients in the proportions as given in the example last mentioned an alloy is produced useful for cable coverings and the like.

The method of compounding the alloy is as 15 follows: The lead is heated to a temperature of approximately 1600° Fahrenheit, that is, so as to raise its temperature somewhat above the melting temperature of calcium, which is 1490° Fahrenheit. The melted lead is covered with a supernatant covering which will not burn at this temperature and which will exclude oxygen and be neutral to the metals to be introduced. The preferred covering consists of calcium chloride. The calcium, aluminum and tin, if tin is used, are introduced 20 into the molten lead under its covering of calcium chloride. The melt is then cooled to a temperature of between 650° to 700° F. and the sodium introduced into the melt. A preferable way, however, is to pour the mixture of 25 lead, calcium, aluminum and tin into molds and allow it to cool and then remelt to temperature of 650° to 750° Fahrenheit and add the sodium. In this case the remelted lead should have a supernatant covering consisting 30 of sodium hydrate (the hydrate of another alkali metal, as potassium, might be used) and rosin, or soap, fuel-oil or other organic substance which will exclude oxygen.

35 40 The final mixture is then poured into ingots.

I claim:

1. An alloy consisting principally of lead and containing sodium in an amount not in 45 excess of 1.0% by weight; calcium 0.1% to 0.25%; and aluminum 0.02% to 0.1%.
2. An alloy consisting principally of lead and containing tin in an amount from 1.0% to 5.0% by weight; sodium not in excess of 50 1.0%; calcium 0.1% to 0.25%; and aluminum 0.02% to 0.1%.
3. An alloy consisting principally of lead and containing sodium not in excess of 0.7% by weight; calcium 0.1% to 0.25%; and aluminum 55 0.02% to 0.1%.

ROBERT JAY SHOEMAKER.